

July 24, 1962

W. F. HAFNER ET AL  
METHOD OF PREPARING IMPROVED WOOD PRESERVATIVE  
FROM COAL TAR CREOSOTE  
Filed May 15, 1959

3,046,217



INVENTORS  
WILLIAM F. HAFNER  
CHARLES W. LEACH  
THOMAS W. SMEAL  
BY  
Donald G. Dalton

ATTORNEY

# United States Patent Office

3,046,217

Patented July 24, 1962

1

3,046,217

## METHOD OF PREPARING IMPROVED WOOD PRESERVATIVE FROM COAL TAR CREOSOTE

William F. Hafner, Monroeville, Charles W. Leach, Trafford, and Thomas W. Smeal, Jeannette, Pa., assignors to United States Steel Corporation, a corporation of New Jersey

Filed May 15, 1959, Ser. No. 813,515

2 Claims. (Cl. 208—2)

This invention relates to a method of preparing an improved wood preservative from coal tar creosote.

Conventional coal tar creosote forms an excellent wood preservative, but its dark color and strong odor restrict its use; an object of our invention is to provide a method of preparing an improved wood preservative from coal tar creosote processed to lighten its color and lessen its odor without impairing its preservative properties.

A more specific object is to provide a method of preparing an improved wood preservative by oxidizing impurities normally present in coal tar creosote, separating oxidized impurities by distillation, and filtering crystalline materials from the distillate, leaving a light-colored preservative of mild odor.

A further object is to provide an improved method of preserving wood in which a wood body is impregnated with a preservative prepared in the foregoing manner.

Other objects are to provide an improved preservative from coal tar creosote which is light-colored and of only mild odor, and an improved wood product resulting from impregnation therewith.

In the drawing:

The single FIGURE is a schematic flowsheet showing the steps of our method.

We prepare our improved wood preservative from conventional coal tar creosote which has a minimum boiling point of about 230° C. and possesses the usual murky brown color and strong odor. First we heat such creosote to about 100–150° C. While the creosote is maintained at this temperature, we introduce streams of air thereto at a rate of about 60 to 100 standard cubic feet per minute per ton of creosote for at least one hour. Some of the more easily oxidized saturated cyclic compounds in the creosote oxidize and form stable oxidation products. After the air-blowing step, the color of the creosote changes to a dull black. As a separate step, we then distill the air-blown creosote under a vacuum, preferably equivalent to about 60 mm. of mercury, to an end temperature equivalent to an end temperature of about 395–410° C. at atmospheric pressure. The oxidized impurities remain as residue, while the purified creosote is the distillate. We consider it necessary to perform the air-blowing and vacuum distillation steps separately, since performing them simultaneously would not permit sufficient contact time with the air. Next we cool the distillate to a maximum temperature of about 40° C., thereby forming crystals rich in anthracene-phenanthrene-carbazol. Finally we remove these crystals by a filtration or equivalent step, recovering our completed preservative as filtrate. The drawing shows the foregoing steps only schematically, since the individual pieces of apparatus are conventional.

The resulting preservative is only lightly colored, and if desired it can be dyed various shades. The odor is mild. A wood body can be impregnated with our preservative by any standard procedure. The resulting wood product is durable and has a light pleasing color and mild scent. Crystals recovered in the filtration step also are a valuable by-product.

2

## Example 1

As a specific example to illustrate our method, we selected as starting material a sample of coal tar creosote having the following physical characteristics:

|    |                                                      |        |
|----|------------------------------------------------------|--------|
| 5  | Specific gravity 38/15.5° C.                         | 1,1014 |
|    | Percent of crystals at 38° C.                        | 11.4   |
|    | Creosote's distillation pattern<br>(AWPA A1-57*) to— |        |
| 10 | 210° C. percent                                      | 0.0    |
|    | 235° C. do                                           | 0.3    |
|    | 270° C. do                                           | 8.5    |
|    | 315° C. do                                           | 40.9   |
|    | 355° C. do                                           | 71.0   |
| 15 | 400° C. do                                           | 90.0   |
|    | Residue do                                           | 9.4    |
|    | Loss do                                              | 0.6    |
|    | First drop ° C.                                      | 233    |

\* American Wood-Preserver's Association, "Manual of Recommended Practice," Subject Designation A1-57.

This sample was air-blown (air at room temperature) for 1½ hours with an air flow rate equivalent to 80 s.c.f.m. per ton of creosote. During this operation, the temperature of the creosote rose from 135° C. to 165° C. The color of the creosote after being air-blown was a dull black (compared to the original murky-brown color), indicating the formation of objectionable compounds.

25 A sample of this air-blown creosote was then redistilled as follows:

|    | Distillation temp., ° C., to— | Distillate, percent of original weight |
|----|-------------------------------|----------------------------------------|
| 35 | 210                           | 0.0                                    |
|    | 235                           | 0.0                                    |
|    | 270                           | 4.3                                    |
|    | 315                           | 35.8                                   |
|    | 355                           | 69.8                                   |
| 40 | 400                           | 87.4                                   |
|    | Residue                       | percent                                |
|    |                               | 12.2                                   |
|    | Loss                          | do                                     |
|    |                               | 0.4                                    |
|    | First drop                    | ° C.                                   |
|    |                               | 251                                    |

45 The residue above 400° C. from this distillation was discarded. The 235 to 400° C. fraction was then vacuum-filtered through a 200-mesh sieve at 38° C., removing 15.0 percent by weight of the original creosote in the form of crystals.

50 The creosote produced by these operations was a clear oil with a light-yellow color and having little of the characteristic odor of creosote. It represented 72.8 percent by weight of the starting material, was crystal-free at 38° C., and had the following distillation pattern (AWPA A1-57).

|    | Distillation temp., ° C., to— | Distillate, percent of original weight |
|----|-------------------------------|----------------------------------------|
| 60 | 210                           | 0.0                                    |
|    | 235                           | 0.0                                    |
|    | 270                           | 6.6                                    |
|    | 315                           | 43.0                                   |
|    | 355                           | 77.0                                   |
| 65 | 400                           | 94.9                                   |
|    | Residue                       | percent                                |
|    |                               | 4.6                                    |
|    | Loss                          | do                                     |
|    |                               | 0.5                                    |
|    | First drop                    | ° C.                                   |
|    |                               | 247                                    |

70 Soil-block bioassay and permanence studies indicated that this creosote had wood-preserving properties as good as, or slightly better than, AWPA grade 1 creosotes.

## Example 2

A sample of creosote, identical with the starting material in Example 1, was air-blown (air at room temperature) for 4½ hours with an air flow rate equivalent to 80 s.c.f.m. per ton of creosote. During the operation, the temperature of the creosote rose from 120° C. to 172° C. The color of the creosote after being air-blown was a dull black (compared to the original murky-brown color), indicating the formation of objectionable compounds.

A sample of this air-blown creosote was then redistilled as follows:

| Distillation temp., ° C., to— | Distillate, percent of original weight |
|-------------------------------|----------------------------------------|
| 210                           | 0.0                                    |
| 235                           | 0.0                                    |
| 270                           | 1.4                                    |
| 315                           | 29.1                                   |
| 355                           | 64.6                                   |
| 400                           | 80.6                                   |
| Residue                       | percent                                |
| Loss                          | do                                     |
| First drop                    | ° C.                                   |

The residue above 400° C. from this distillation was discarded. The 235 to 400° C. fraction was then vacuum-filtered through a 200-mesh sieve at 38° C., removing 13.1 percent by weight of the original material in the form of crystals.

The creosote produced by these operations was a clear oil with a light-yellow color and having little of the characteristic odor of creosote. It represented 67.9 percent by weight of the starting material, was crystal free at 38° C., and had the following distillation pattern (AWPA A1-57):

| Distillation temp., ° C., to— | Distillate, percent of original weight |
|-------------------------------|----------------------------------------|
| 210                           | 0.0                                    |
| 235                           | 0.0                                    |
| 270                           | 2.8                                    |
| 315                           | 37.4                                   |
| 355                           | 73.9                                   |
| 400                           | 92.9                                   |
| Residue                       | percent                                |
| Loss                          | do                                     |
| First drop                    | ° C.                                   |

Soil-block bioassay and permanence studies indicated that this creosote had wood-preserving properties as good as, or slightly better than, AWPA grade 1 creosotes.

From the foregoing description and examples it is seen that our invention affords a simple method of preparing an improved wood preservative from coal tar creosote, but eliminating objectionable color and odor. Our preservative retains all the desirable characteristics of conventional creosote, and the absence of crystalline substances permits easier transfer through pipes and pumps, lessens the heat required to maintain fluidity, and facilitates the impregnation process.

While we have shown and described certain preferred ways of practicing our invention, it is apparent that other modifications may arise. Therefore, we do not wish to be limited to the disclosure set forth but only by the scope of the appended claims.

We claim:

1. A method of preparing a refined creosote from coal tar creosote which has a minimum boiling point of about 230° C. comprising heating said coal tar creosote to about 100-150° C., introducing an air stream to the heated coal tar creosote at a rate of about 60 to 100 standard cubic feet per minute per ton of coal tar creosote for at least one hour and thus oxidizing unsaturated cyclic compounds present in the coal tar creosote and forming stable oxidation products, as a separate step distilling the coal tar creosote under vacuum to an end temperature corresponding to an end temperature of about 395-410° C. at atmospheric pressure and thus separating a creosote product as distillate and said oxidation products as residue, cooling said distillate to a maximum temperature of about 40° C., and filtering said cooled distillate to remove crystals rich in anthracene-phenenathrene-carbazol, thus recovering a refined creosote having a light color and mild odor.

2. A refined creosote prepared according to the method defined in claim 1.

## References Cited in the file of this patent

## UNITED STATES PATENTS

|           |               |               |
|-----------|---------------|---------------|
| 1,037,832 | Newton        | Sept. 3, 1912 |
| 2,066,583 | Shipley       | Jan. 5, 1937  |
| 2,095,190 | Heuscher      | Oct. 5, 1937  |
| 2,246,973 | Camilli       | June 24, 1941 |
| 2,655,454 | Farber et al. | Oct. 13, 1953 |
| 2,864,846 | Gragson       | Dec. 16, 1958 |